

## UNITED STATES PATENT OFFICE

2,304,157

## PROCESS FOR IMPROVING TEXTILES

Max Engelmann, Wilmington, Del., and Josef Plik, Pitman, N. J., assignors to E. I. du Pont de Nemours & Company, Wilmington, Del., a corporation of Delaware

No Drawing. Application October 2, 1940,  
Serial No. 359,360

13 Claims. (Cl. 8—116)

This application is a continuation-in-part of our copending application Serial No. 322,766, filed March 7, 1940, and relates to a process for treating fibrous materials to modify their surface characteristics.

It is an object of this invention to provide a process for imparting water-repellency and softness of feel to fibrous material of vegetable, animal or synthetic origin, using the novel phosphonic acid compounds described and claimed in said copending application. Other and further important objects of this invention, will appear as the description proceeds.

In our copending application, Serial No. 322,766, above referred to we have described a series of novel organic compounds which may be designated generally as acyl-amido-methylene phosphonic acids. They are synthesized from methylol-amides of carboxylic acids by reacting upon the latter with a phosphorus trihalide to produce an intermediate phosphorus halide compound, and then decomposing the latter by water (or atmospheric humidity) to give a phosphonic acid. The general scheme of synthesis and the resulting products is typified by the following equations:



In these formulas, R' stands for hydrogen or a lower alkyl radical, while R designates any organic radical whatsoever which is linked to the N atom through the keto group (CO) or the thione group (CS). Thus, R may stand for the group-



wherein R'' may be an aliphatic, cycloaliphatic, or aromatic radical, which may carry various substituents, for instance halogen, the carboxyl group or sulfonic acid radicals. Or R may take

the form R''—O—CO, R''—NH—CO, R''—CO—NH—CO, R''—O—CO—NH—CO, etc., wherein R'' is a long-chain aliphatic radical.

As a special subgroup under the above general formulas come into consideration those compounds wherein R contains an aliphatic or cycloaliphatic radical of at least 10 carbon atoms. The members of this subgroup have the common property of modifying the surface characteristics of textile fibers, bestowing upon the same a soft feel and the quality of water-repellence. Depending upon the mode of treatment, both of these properties can be rendered substantially permanent in the sense that the effect is not substantially impaired by laundering and dry-cleaning.

The method of synthesis of the novel compounds has been described in detail in our parent application above referred to, and therefore need not be taken up in detail here.

Our present invention is concerned primarily with the utilization of these novel compounds for the purpose of modifying the surface characteristics of fibrous materials. We have found that the above special group of compounds which are obtained from amides having an aliphatic or cycloaliphatic radical, in their structure, of from 10 to 28 carbon atoms are very active as softening agents and water-repellency agents for textile fiber. Moreover, although but sparingly soluble in the form of free phosphonic acid, they may be readily converted into water-soluble salts by neutralization of the phosphonic OH groups, individually or jointly, with alkali-metal hydroxides, or with ammonia and organic amines. In a number of cases, we have actually prepared and isolated the sodium, ammonium, diethanolammonium and pyridinium salts.

These salts, especially the ammonium salts, are very convenient agents for application to the fiber from an aqueous bath. However, it is not necessary to prepare and isolate these salts in substance, inasmuch as it is sufficient to dissolve the free phosphonic acids in an aqueous bath containing an inorganic or organic base, for instance sodiumhydroxide, ammonia, pyridine or mono-, di- or triethanolamine. Moreover, good results may also be obtained by using the free phosphonic acids in the absence of alkalies, inasmuch as the solubility of these acids is often as high as 1%. Depending on the concentration of the bath, the fiber may be endowed with a soft feel or with both softness and water-repellency. A concentration of 0.5 to 5% by weight of the aqueous bath will generally give satisfactory results for

water-repellency plus incidental softness, while for softness alone even a concentration as low as 0.01% has been found effective.

The treatment generally consists of impregnating the fiber with the aqueous bath at room temperature or slightly elevated temperature, say up to 45 or 50° C. The fiber is then squeezed out or centrifuged until it retains just about its own weight of the impregnating solution. It is then optionally dried at a temperature, say, below 70° C., and then subjected to a baking treatment at a temperature between 90 and 200° C., preferably between 100 and 170° C., for a period of time which varies somewhat inversely with the temperature as more fully explained hereinbelow.

In the case of treatment for softness alone, we have found it advantageous to subject the fabric after baking to a soaping treatment in an aqueous bath containing a true soap, that is an alkali-metal or equivalent salt of a fatty acid. A concentration of 0.1 to 1% of the soap has been found by us satisfactory for this purpose.

Without limiting our invention to any particular procedure, the following examples are given to illustrate our preferred mode of operation. Parts mentioned are by weight.

#### Example 1

100 parts of methylol stearamide were added to a mixture of 45 parts of carbon tetrachloride and 91 parts of phosphorus trichloride. One hour after all the methylol amide had been added, 40 parts of acetic acid were added and the reaction mass was allowed to stand at room temperature for four days. The reaction mixture gradually became a viscous mass and at the same time soluble in dilute alkalies. The product was decomposed with 8% hydrochloric acid at about 50° C. and yielded a crystalline readily filterable product which could be recrystallized from alcohol. It meted to an opaque mass at about 108° C., but did not become completely homogeneous until heated to a much higher temperature. It was readily soluble in dilute alkalies and in hot water giving a viscous foaming solution.

When cotton was treated with an aqueous solution of the ammonium salt of this phosphonic acid and then heated to 150° C. for a few minutes, the fabric acquired a very soft feel and was strongly water-repellent. These properties were not lost when the fabric was washed.

#### Example 2

30 parts of methylol stearamide were suspended in 300 parts of ethyl acetate and at 25° C. 17 parts of phosphorus tribromide added. When the reaction mass was warmed to 40° C. a clear solution resulted. It was held at 40 to 45° C. for two hours then allowed to cool to room temperature. After 14 hours a crystalline product had separated which was filtered off, decomposed with water and crystallized from alcohol. The product was identical with the compound prepared according to Example 1, and produced upon cotton the same effect.

#### Example 3

45 parts of methylol amide from a mixture of carboxylic acids having 20 and 22 carbon atoms was added to 100 parts of phosphorus trichloride at room temperature and agitated for 1 hour. 38 parts of acetic acid was added and then allowed to stand at room temperature for 3 days. The hard reaction product was broken up and decomposed by ice and then filtered. The product dissolved in methyl alcohol on warming to an al-

most clear solution and crystallized again on cooling. The product was soluble in water containing a small amount of a base like NaOH, ammonia or pyridine.

When a piece of cotton cloth was padded in a 2% solution of this product in water containing 0.5% ammonia and then heated for 5 minutes to 150° C. the cloth became water-repellent and acquired a soft feel. Both properties were stable towards washing.

#### Example 4

Naphthenic acid amide was converted into the corresponding methylol compound by reacting the amide with formaldehyde in an alcoholic solution.

32 parts of the oily methylol naphthene amide were mixed with 27 parts of  $PCl_3$  and 24 parts of acetic acid and then allowed to stand at room temperature for several days. The reaction mass was decomposed with ice and the oily bottom layer taken up with petroleum ether. Upon evaporation of the solvent a thick orange colored oil was left which was soluble in warm water and in dilute alkalies. It contained the expected amount of phosphorus and nitrogen. This product exhibited strong antioxidant and metal-deactivating properties, deactivating metals such as iron, manganese, cobalt and copper.

When an ammoniacal solution was applied to cotton or rayon and the cloth heated for a few minutes to temperature of 120° to 170° C. it became water-repellent and soft but not as marked as when treated with products of Example 1.

#### Example 5

32 parts of hydroabietic acid methylol amide were added at room temperature to 30 parts of phosphorus trichloride, and 16 parts of acetic acid were added and the reaction mass allowed to stand at room temperature for several days. The originally thin mass gradually became a hard product which could not be stirred. When the reaction was completed the condensation product was treated with 250 parts of water, and the pasty product was taken up with ether. Upon evaporation of the ether a hard mass remained which could be pulverized. It was soluble in dilute alkalies and had strong foaming properties.

When an ammoniacal solution was applied to cotton or rayon and the cloth heated for a few minutes to temperature of 120 to 170° C., it became water-repellent and soft but not as marked as when treated with products of Example 1.

#### Example 6

50 parts of methylol octadecyl carbamate as prepared according to French Patent No. 840,002 were added to 160 parts of phosphorus trichloride at room temperature. After agitating for 1 hour, 38 parts of acetic acid were added and the reaction mass allowed to stand at room temperature for several days. The hard reaction mass was broken up, decomposed by ice and then filtered. By purification with methyl alcohol a small amount of an insoluble material was removed. The main fraction was very soluble in dilute aqueous ammonia. The analysis corresponded to that of the expected compound of the formula



When applied to cotton in the way as described in Example 1, it imparted to the fabric a strongly

water-repellent, soft finish. Instead of the methyol octadecyl carbamate an equivalent amount of another carbamate of a higher or lower molecular weight may be used, such as the corresponding tetradearyl carbamate, hexadecyl carbamate, or octadecyl-phenyl carbamate.

*Example 7*

8 parts of the dimethylol amide of methylene distearamide, which was prepared by decomposing methylene-bis-(stearamidomethyl-chloride) (British Patent No. 517,474) with 50%  $K_2CO_3$  at low temperature, were added to 20 parts of  $PCl_3$  at room temperature. To the clear thin solution which was obtained in a few minutes, 5 parts of acetic acid were added. Upon standing at room temperature over night, the mass solidified to a very thick plastic mass which dissolved in ammoniacal water to a clear solution.

The product was decomposed with water and then purified by dissolving it in dilute ammonia, filtering out some insoluble material and precipitating the phosphonic acid from the alkaline solution with hydrochloric acid. In this way a product was secured which dissolved to a perfectly clear solution in warm water containing a small amount of a base.

Cotton cloth and rayon taffeta were impregnated with a 1% solution of the ammonium salt of this phosphonic acid and then heated to 150° C. for a few minutes. After this baking treatment the goods were washed with sodium oleate soap and dried. Both samples showed a very soft feel and a strong water-repellency.

The dimethylol amide used as initial material in this example is a new compound and is further described and claimed in copending application of Josef Píkl, Serial No. 362,730.

*Example 8*

10 parts of the product prepared according to Example 1 was dissolved in 1000 parts of water with the aid of some ammonia. Cotton broad cloth was impregnated with this solution and dried for 10 minutes at 165° C. then washed for five minutes at 180° C. in a 0.5% solution of sodium oleate and finally rinsed in hot water, and dried.

The cloth acquired a very soft feel.

*Example 9*

Viscose process rayon yarn was impregnated with a solution of stearamidomethyl phosphonic acid (Example 1) containing 0.1 part of the product per liter; the yarn was then dried at room temperature and heated for 5 minutes to 140° C.

After the baking, the yarn had a soft touch but showed only a little water-repellency. It was now washed for 15 minutes in  $\frac{1}{2}\%$  solution of oleic-acid soap and rinsed in hot water. The softness of the yarn was greatly improved by this washing treatment.

It will be understood, that although our specific examples above dealt particularly with the treatment of cotton and rayon, this invention is applicable also to the waterproofing of animal fibers, such as wool, silk, leather; of synthetic fiber, such as regenerated cellulose, nylon; and to non-fibrous cellulosic films, such as Cellophane. Furthermore, the details of procedure may be varied within wide limits without departing from the spirit of this invention.

Thus, the concentration of the amido-methylene phosphonic acid salt in the treatment bath may vary from 1 to 8% by weight. A good rule to follow is to use such a concentration that

5 after impregnation and squeezing out excess moisture, the fiber shall contain the ether in from 1 to 4% of its own weight. Thus, if the fiber is squeezed until it contains its own weight of moisture, the concentration of the bath may be from 1 to 4%. But if the fiber is squeezed until the pick-up is only 50% of its dry weight, the initial concentration of the treatment bath should be twice as high.

10 Formaldehyde, dimethylol urea or other agents yielding formaldehyde in aqueous solution may be added to the bath to increase its effectiveness and the permanence of the resulting treatment, in accordance with copending application of O. C. Bacon, Serial No. 336,375. The quantity added may vary from 0 to 3% by weight of the total bath. Higher concentrations may be employed, provided a tertiary amine is employed instead of ammonia for solubilizing the phosphonic acid.

15 The temperature of impregnation may be varied from room temperature to about 45° or 50° C. Lower or higher temperatures may be used, but there is no apparent advantage.

20 As already indicated, the intermediate drying step may be employed or omitted, since the presence of moisture during the baking treatment is not so critical here as in the case of octadecyloxy-methyl-pyridinium chloride, for instance.

25 The baking temperature may vary from 90 to 200° C. but is usually more conveniently selected between 100 and 170° C. The time required for baking varies somewhat inversely with the temperature, and may be as high as 30 minutes at the lower temperature limit and as low as  $\frac{1}{2}$  minute at the higher limit. The optimum time for any given reagent and temperature combination may be determined experimentally by 30 treating samples of the chosen fabric and then estimating, by the usual tests, the intensity and durability of the water-repellent effect bestowed on it. Time periods in excess of the optimum do not affect the water-repellency, but tend to weaken the fiber, in the case of cellulose, due to exposure to the acids liberated in the baking step.

35 In other details, our novel process may follow in general the hitherto established processes for waterproofing fiber with quaternary ammonium compounds as typified by cetylxy-methyl pyridinium chloride and stearamido-methyl pyridinium chloride.

We claim:

1. A process for treating textile fiber for the purpose of modifying the surface characteristics thereof, which comprises impregnating the same with a compound selected from the group consisting of the free methylene-phosphonic acid selected from the group of compounds corresponding to the formulas—



and



wherein R' stands for a substituent of the group consisting of hydrogen and lower alkyl, while R is an organic radical containing a chain of not less than 10 carbon atoms, but being free from water-solubilizing groups and being attached to the N-atom through the agency of a ketonic link selected from the group consisting of C=O and

$\text{C}=\text{S}$ ; and then subjecting the impregnated fiber to the action of heat at a temperature between 90 and 200° C.

2. A process as in claim 1 including further the step of subjecting the fiber after heat-treatment to the action of an aqueous bath containing a soap of a fatty acid.

3. A process for treating textile fiber for the purpose of modifying the surface characteristics thereof, which comprises impregnating the same with a water-soluble salt of an amido-methylene-phosphonic acid selected from the group of compounds corresponding to the formulas—



and



wherein  $\text{R}'$  stands for a substituent of the group consisting of hydrogen and lower alkyl, while  $\text{R}''$  is an organic radical containing a saturated carbon chain of not less than 10 carbon atoms, but being free from water-solubilizing groups; and then subjecting the impregnated fiber to the action of heat at a temperature between 90 and 200° C.

4. A process as in claim 3 including further the step of subjecting the fiber after heat-treatment to the action of an aqueous bath containing a soap of a fatty acid.

5. A process for treating textile fiber for the purpose of modifying the surface characteristics thereof, which comprises impregnating the same with a salt of an amido-methylene-phosphonic acid of the general formula



wherein  $\text{R}$  is an organic radical containing a saturated carbon chain of not less than 10 carbon atoms, but being free from water-solubilizing groups; and then subjecting the impregnated fiber to the action of heat at a temperature between 90 and 200° C.

6. A process for treating textile fiber for the purpose of modifying the surface characteristics thereof, which comprises impregnating the same with a salt of an amido-methylene-phosphonic acid of the general formula



wherein  $\text{R}$  is a radical selected from the group consisting of aliphatic and cycloaliphatic radicals having from 10 to 28 carbon atoms and being free from water-solubilizing groups,  $\text{Y}$  is an atomic bridge selected from the group consisting of  $\text{CH}_2$ ,  $\text{O}$ ,  $\text{S}$ ,  $\text{NH}$  and  $\text{CONH}$ ; and then subjecting the impregnated fiber to the action of heat at a temperature between 100 and 170° C.

7. A process for treating cellulosic textile fiber for the purpose of modifying the surface characteristics thereof, which comprises impregnating

the same with an aqueous solution of a salt of an amido-methylene-phosphonic acid of the general formula  $\text{Alk}-\text{CONH}-\text{CH}_2-\text{PO}(\text{OH})_2$ , wherein  $\text{Alk}$  designates an alkyl radical of from 10 to 28 carbon atoms; removing excess moisture, and then subjecting the fiber to a heat treatment at a temperature between 100 and 170° C. for a period of time sufficient to cause decomposition of said amido-methylene phosphonic acid compound.

8. A process as in claim 5, wherein the aqueous solution employed for impregnation contains said amido-methylene-phosphonic acid compound in a concentration of from 0.5 to 5% by weight.

9. A process as in claim 5, wherein the aqueous solution employed for impregnation contains said amido-methylene-phosphonic acid compound in a concentration of from 0.01 to 0.5% by weight, the heat treatment being followed by a soaping treatment of the fiber in an aqueous solution of a fatty acid soap.

10. A process for treating cellulosic fiber for the purpose of modifying the surface characteristics thereof, which comprises impregnating the same with an aqueous solution of a salt of an amido-methylene-phosphonic acid of the general formula



wherein  $\text{R}$  is an organic radical containing an aliphatic or cycloaliphatic group of from 10 to 28 carbon atoms; removing excess moisture, and then subjecting the fiber to a heat treatment at a temperature between 100 and 170° C. for a period of time sufficient to cause decomposition of said amido-methylene phosphonic acid compound.

11. In a process of treating textile fiber to render the same water-repellent, the step which consists of impregnating the same with an aqueous solution of the ammonium salt of stearamido-methylene-phosphonic acid, and then heating the fiber in the absence of moisture to decompose said agent on the fiber.

12. In a process of treating textile fiber to render the same water-repellent, the step which consists of impregnating the same with an aqueous solution of the ammonium salt of methylene-bis-(stearamido-methylene-phosphonic acid), and then heating the fiber in the absence of moisture to decompose said agent on the fiber.

13. In a process of treating textile fiber to endow the same with a soft feel, the improvement which consists of impregnating the same with an aqueous bath containing stearamido-methylene-phosphonic acid, and then heating the fiber in the absence of moisture to decompose said agent on the fiber.

MAX ENGELMANN.  
JOSEF PIKL.